

## UNITED STATES PATENT OFFICE

2,583,200

## NONSPREADING LUBRICANT

George E. Barker, Newport, Del., assignor to Elgin National Watch Company, Elgin, Ill., a corporation of Illinois

No Drawing. Application March 8, 1946;  
Serial No. 653,124

10 Claims. (Cl. 252—57)

1

This invention relates to non-spreading lubricants which are of particular value under conditions of boundary lubrication. By "boundary lubrication" is meant the condition of operation between two relatively movable parts, with a lubrication film interposed therebetween and with the parts moving at such low relative speeds that the forces of adhesion between the lubricant and the parts determine the maintenance of the lubrication film against the action of the forces which are tending to bring the parts together. An example of such behavior occurs in fine instruments such as watches, meters, etc., where pivot staffs turn in jewel bearings at low rates of speed, and in which for accuracy of movement of indication, the frictional resistance must be kept low and substantially uniform.

In my granted Patent 2,355,616 I have described the employment of organic substances as lubricants which are effective under boundary lubrication conditions, and which demonstrate a high contact angle to normal bearing surfaces of fine instruments, that is, while such lubricants are in contact with brass, steel, ruby, etc. In the said patent reference has been made to the desirability of employing mixtures of homologs in order to keep the solidifying point low, so that the lubricant will be effective down to low temperatures; these homologs being substances of related properties and each having a high contact angle effect.

It has now been found that under certain restricted conditions it is feasible to employ mixtures of such non-spreading lubricants with organic compounds which individually are of spreading type or which have extremely low contact angles relative to brass, steel, ruby, etc., such contact angles being of the order of 5 degrees or less under the conditions of determination and measurements set out in my aforesaid patent. An example of this has been set out in the Barker application Serial No. 547,979 filed August 3, 1944, now U. S. Patent No. 2,412,956, granted December 24, 1946; of which the present application is a continuation-in-part.

The effect of such mixtures of non-spreading and spreading lubricants is to produce a lubrication medium which has superior properties as compared with the individual components, and having in many instances superiority over the corresponding individual values for each of the components.

The limitation upon employment of such spreading diluents for a non-spreading lubricant is that the diluent should consist of organic com-

pounds or mixtures of homologous organic compounds, in which each compound has two groups of which one is an ester group and the other may be either an ester or an aryl group. The mixture must be substantially free of the normal mineral oils, of which a maximum of up to 5 percent may be tolerated by some such mixed lubricants: this content of mineral oil must take into account not only the presence of impurities in the lubricant as prepared for use, but also the presence of such mineral oils by reason of their employment in forming or machining the parts to be lubricated and the possible presence from prior employment as lubricant therebetween. As set out in my aforesaid patent, it is therefore at least advisable to perform thorough cleaning operations upon the parts before bringing them together in the presence of the non-spreading lubricant medium. As a corollary, the instant lubricants are clearly and definitely to be distinguished from any employment of additives for modifying or improving the behavior of a mineral oil lubricant.

## Example I

25 As a specific example of practice, a lubricant prepared from 60 parts by weight of benzyl phenylundecanoate, 40 parts of diethylene glycol dicaproate, 0.5 part dodecylpiperidine stearate and 0.1 part of tertiary-butyl catechol, has a viscosity (centistokes) of 10.2 at 100 degrees F., and 53.6 at 32 degrees F.; a pour point of minus 70 degrees F.; no corrosion on brass or steel; a surface tension of 36.0 dynes per centimeter; contact angles of 25 degrees on brass, 21 degrees on steel and 23 degrees on ruby; and having an evaporation factor of 81 percent. (This evaporation factor is the percentage of a 1.0000 gram sample remaining after 100 hours at 70 degrees C., or the equivalent 158 degrees F., while passing dry nitrogen gas through the oil at the rate of  $\frac{1}{2}$  cubic foot per hour in a cell which assures essential saturation of the gas with oil vapor.)

40 By way of comparison, the employed benzyl phenylundecanoate itself has a viscosity of 17.6 centistokes at 100 degrees F. and 142.5 at 32 degrees F.; a pour point of minus 40 degrees F.; no corrosion on brass; a surface tension of 39.5 dynes per centimeter; and a contact angle of 19 degrees on steel. This ingredient is a composition including homologs with a boiling range of 195 to 210 degrees C. at one mm. pressure, where-with the viscosity may vary for various specimens, but the values of 17.0 to 17.7 at 100 degrees F. essentially covers the range. Thus, this substance of itself is a non-spreading compound

which can be used for boundary lubrication, but has the difficulty of a large change in viscosity and a high minimum pour point (minus 40 degrees F.) which unfit it for employments where a low viscosity-temperature factor and operativeness at minus 60 degrees F. or below are requisite.

Diethylene glycol dicaprate was used in the form of homologs having a boiling range of 149 to 162 degrees C. at one mm. Of itself it is a spreading lubricant; the viscosity is around 5.3 centistokes at 100 degrees F. and 18.6 at 32 degrees F. Its cloud and pour points are at minus 2 degrees F. (crystallization) and hence it freezes under conditions of airplane service of fine instruments. It exhibits no corrosion against brass, and has a surface tension of around 32.9 dynes per centimeter.

It is striking that this mixture exhibited a contact angle effect against steel, for example, which is greater than that of any component, whereas a mixture of the benzyl phenylundecanoate with, say, 5 percent of mineral oil lubricant, spreads essentially with the same ease as the mineral oil itself. It is likewise striking that the pour point of this mixture is well below the pour point of either of these constituents. Furthermore, the viscosity shift between 100 degrees F. and 32 degrees F. is of the order of 1:5; whereas the benzyl phenylundecanoate component has a factor of around 1:7 and the diethylene glycol dicaprate component has a factor of around 2:7.

The dodecylpiperidine stearate is introduced to improve the coefficient of friction during service as set out in my co-pending application, Serial No. 547,979, filed August 3, 1944, in which the employment of alkyl piperidine salts for such purposes is claimed.

The tertiary butyl catechol is included as a stabilizing or anti-oxidizing agent to offset minor tendencies toward oxidation by the presence of the ester groupings in the major ingredients.

#### Example II

70 parts by weight of the same benzyl phenylundecanoate, 30 parts of diethylene glycol divalerate, 0.2 part of tri-isobutyl phenol and 0.2 part of stearic acid, with the major ingredients in the form of mixtures of homologs, provides a non-spreading lubricant having viscosity of 10.4 centistokes at 100 degrees F. and 57.7 centistokes at 32 degrees F.; a pour point of minus 65 degrees F.; no corrosion on brass or steel; a surface tension of 35.8 dynes per centimeter; contact angles of 29 degrees on brass; 9 degrees on steel and 25 degrees on ruby; and an evaporation factor of 69 percent. This material is therefore useful within a lesser minimum and maximum temperature range than the material of Example I, and with a slightly lower surface tension value.

With respect to the properties of the diethylene glycol divalerate component, this ingredient has a boiling range of 128-130 degrees C. at 0.5 mm.; a viscosity of 3.8 centistokes at 100 degrees F. and 12.5 at 32 degrees F.; a pour point of minus 90 degrees F.; no corrosion on brass; and a surface tension of 31.7 dynes per centimeter. It is noteworthy that the pour point of this diester is below that of the corresponding dicaprate ester of Example I, but the mixture of ingredients does not reveal a corresponding depression of pour point.

#### Example III

50 parts by weight of the same benzyl phenylundecanoate, 50 parts of methyl phenylundecanoate, and 0.1 part of oleic acid, with the major

ingredients composed of homologs as before, provides a mixture having a viscosity of 12.3 centistokes at 100 degrees F. and 78.5 at 32 degrees F.; and contact angles of 23 degrees on brass, 12 degrees on steel, and 28 degrees on ruby. This composition is illustrative in that the benzyl ester is non-spreading while the corresponding methyl ester spreads. This methyl ester had a boiling range of 150 degrees to 175 degrees C. at one mm., a viscosity of 9.1 centistokes at 100 degrees F. and 48.5 at 32 degrees F.; a pour point of minus 70 degrees; no corrosion on brass or steel; and a surface tension of 35.8 dynes per centimeter. This methyl ester satisfies the specification above in that it has two groups including the ester grouping between the methyl alcohol and the phenylundecanoic acid, and the second group is provided by the phenyl radical which is an aryl group.

#### Example IV

90 parts by weight of the same benzyl phenylundecanoate, 10 parts of benzyl undecanoate, 0.1 part of tri-isobutyl phenol, and 0.1 part of stearic acid, provides a mixture in which the major ingredients are composed of homologs as before, and has a viscosity of 15.9 centistokes at 100 degrees F. and 93.5 at 32 degrees F.; a pour point of minus 50 degrees F.; no corrosion on brass or steel; a surface tension of 38.2 dynes per centimeter; contact angles of 17 degrees on brass, 19 degrees on steel and 24 degrees on ruby; and an evaporation factor of 89 percent.

In this mixture, the benzyl undecanoate has the ester grouping and also has the aryl group provided by the benzyl radical which in this instance is on the alcohol rather than on the acid side of the ester connection. By comparison, this benzyl undecanoate itself is a spreading lubricant. However, the behavior in the presence of even less than 5 percent of a normal mineral oil lubricant is to entirely displace the contact angle behavior so that the substituted mixture becomes spreading even in the presence of the large percentage of benzyl phenylundecanoate.

#### Example V

57 parts by weight of benzyl phenylundecanoate, 43 parts of benzylthioethyl caproate, 0.5 part of dodecylpiperidine stearate, and 0.1 part of tertiary butyl catechol provide a non-spreading lubricant having a viscosity of 10.1 centistokes at 100 degrees F., and 56.4 centistokes at 32 degrees F., pour point minus 60 degrees F., and surface tension of 34.4 dynes/cm. It causes a slight corrosion on brass, but is useful for many employments where low viscosity, low pour point and low surface tension are desired.

#### Example VI

50 parts by weight of benzyl phenylundecanoate, 50 parts of thioglycol dicaprate, 0.5 part of dodecylpiperidine stearate, and 0.1 part of tertiary butyl catechol provide a non-spreading lubricant having viscosity of 10.2 and 51.2 centistokes at 100 and 32 degrees F. respectively, a cloud point of plus 40 degrees F. and a pour point of plus 20 degrees F., with no corrosion on brass. This product is useful where the exposure temperature is high.

#### Example VII

66 parts by weight of benzyl phenylundecanoate, 33 parts of thioglycol di (2-ethyl butyrate), 0.55 part of dodecylpiperidine stearate, and 0.1

part of tertiary butyl catechol provide a non-spreading lubricant having viscosity of 12.9 and 81.0 centistokes respectively at 100 and 32 degrees F., non-corrosive to brass, and having a surface tension of 36.6 dynes/cm.

*Example VIII*

50 parts by weight of benzyl phenylundecanoate, 50 parts of thioglycol dihexoate, 0.3 part of dodecylpiperidine stearate, and 0.1 part of tertiary butyl catechol provide a non-spreading lubricant having viscosity of 10.4 and 57.7 centistokes respectively at 100 and 32 degrees F., a pour point of minus 70 degrees F., slight corrosion on brass and steel, and with contact angle of 26 degrees on brass, 16 degrees on steel, and 31 degrees on ruby.

In the above examples, the feasibility of employing spreading type compounds as diluents and composition-modifiers for non-spreading-type lubricants has been set out by employing benzyl phenylundecanoate as a non-spreading base: wherewith the non-spreading product contains (A) a non-spreading-type component, (B) a spreading-type component; these components being compatible in that they form stable inter-solutions or mixtures. Other non-spreading or (A) components can be substituted, such as the compounds having the characteristics and compositions set out in my aforesaid patent, No. 2,355,616; among such substitutes are preferred those with an ester or ether connection between terminal organic groups, for example benzyl phenylvalerate and phenoxyphenyl cetane.

*Example IX*

50 parts by weight of benzyl phenylvalerate, 50 parts of benzyl thioethyl undecanoate, 0.2 part of triisobutyl phenol, and 0.1 part of stearic acid provide a lubricant having viscosity of 9.1 and 51.8 centistokes respectively at 100 and 32 degrees F., a pour point of minus 50 degrees F., low corrosion on brass (the actual corrosion being probably due to impurity in specific sample tested), surface tension 38.4 dynes/cm., and which was non-spreading on brass (contact angle 31 degrees) and ruby (contact angle 21 degrees), and exhibiting for the samples tested a contact angle of 9 degrees on steel.

*Example X*

50 parts by weight of benzyl phenylvalerate, 50 parts of methyl phenylundecanoate, and 0.1 part stearic acid provide a non-spreading lubricant acceptable for service on brass, steel and ruby.

*Example XI*

50 parts by weight of phenoxyphenyl cetane, 50 parts of trimethylene glycol dioctoate, 0.1 part tertiary butyl catechol, and 0.1 part stearic acid provide a non-spreading lubricant having a pour point of minus 60 degrees F., and being non-corrosive to brass.

*Example XII*

70 parts by weight of phenoxyphenyl cetane, 30 parts of trimethylene glycol dihexoate, 0.1 part tertiary butyl catechol and 0.1 part stearic acid, also provide an acceptable non-spreading lubricant.

In the above examples, the corrosion test was performed by submerging a carefully cleaned and bright instrument brass block 2.5 x 1 x 1 centimeters in size and having an area of 12 square centimeters, in about 10 cubic centimeters of the

oil in a glass vessel: the temperature was maintained at 100 degrees C. for 100 hours while passing oxygen gas saturated with water vapor at 3 bubbles per second (0.2 cubic feet per hour): at the end of test, the lubricant was examined for change of viscosity and appearance, and the surface of the brass block was examined for pitting or other evidence of corrosion and weighed after removing the oil. The viscosity change was not over 10 percent, and the weight loss of the brass block was not over 1 milligram for the products accepted as "non-corrosive": surface staining without essential change of weight occurred in some instances. A second test for corrosion on steel is made by half-immersing a high-grade cleaned steel bearing ball in a 20 cc. beaker containing the lubricant, the beaker being then kept in a sealed vessel containing water to maintain a saturated atmosphere, at room temperature, for a period of several months: "satisfactory" lubricants resist this test for 5 or 6 months. A third test for corrosion on steel is conducted by immersing such a steel ball in the lubricant at 65 degrees C. for one hour; then adding distilled water to displace the main body of oil and leave the ball immersed in the water; and then holding the ball so immersed until more than 10 percent of the surface is covered with rust: a "satisfactory" lubricant must resist for at least 2 days. (By comparison, most uninhibited mineral oils of highly refined types fail in a few hours under this test: some even in a few minutes).

The illustrative mixtures of materials can be defined as being non-volatile compositions including a non-spreading or (A) lubricant ingredient consisting essentially of stable polar aralkyl molecules, each comprising an alkyl chain and a nuclear aromatic radical connected to said chain and including a strong non-anionic negative group, the ingredient demonstrating a positive contact angle with a steel surface in excess of 10 degrees and having surface tension of at least 35 dynes per centimeter; the alkyl chain comprising 5 to 21 carbon atoms when a single aromatic nucleus is present, and comprising 3 to 21 carbon atoms when there are a plurality of aromatic nuclei in the molecule. The spreading-type diluent or (B) component employed was illustratively selected from stable organic compounds which contain at least two polar groups, of which one is the ester group, and another is either a second ester group or an aryl group; so that they may be referred to as having ester-ester or diester connections or ester-aryl connections, with feasibility of employing complexes of aryl-thio ether-ester or similar types. It is preferred to have this (B) component in the form of a stable non-volatile organic compound including the said connections and having a saturated aliphatic chain of 4 to 16 carbon atoms, either without substitutions or side groups or including oxygen or sulfur atoms as ether or ester bonds in the chain or a side group. Thus, some of the illustrative (B) components are glycols having di-ester connections to monovalent acids, and others are mono-esters which include an aryl nucleus.

It is usual, as shown by the above examples, to employ 50 to 90 parts by weight of the non-spreading or (A) component, with 50 to 10 parts of the spreading component.

Each of these major constituents or ingredients is preferably present in the form of a mixture of homologs so that the boiling point of the mixture appears as a range of temperature within

7  
which these similar compounds come over during distillation.

It is preferred to include small percentages (not exceeding substantially 1 percent in all) of modifying agent to improve the oiliness, the coefficient of friction, etc.; but care must be taken to avoid the presence during the service of the lubricant of such an amount of mineral oil lubricant as to modify the behavior of the mixture or in itself to perform lubricating service: this content must never exceed 5 percent and should be kept as low as possible, and hence the compositions can be described as essentially free of mineral oil.

It is obvious that the invention is not limited to the forms of practice described, but that the same may be employed in many ways within the scope of the appended claims.

I claim:

1. A non-spreading lubricant having a base consisting of 50 to 90 parts by weight of a non-spreading component and 50 to 10 parts of a spreading component, said components being compatible and intersoluble in one another; said non-spreading component consisting of a liquid homologous mixture of stable non-volatile polar aralkyl compounds each having an alkyl chain and a nuclear aromatic radical connected to said chain and including a strong non-anionic negative group, demonstrating a positive contact angle with a steel surface in excess of 10 degrees and having a surface tension of at least 35 dynes per centimeter, the alkyl chain having from about 5 to 21 carbon atoms; said spreading component consisting of a liquid mixture of stable non-volatile organic compounds each containing a saturated aliphatic chain of 4 to 16 carbon atoms and at least two polar groups, of which one is the ester group and another is selected from the radicals consisting of the ester group and the aryl groups; said lubricant being further characterized in containing less than 5 per cent of mineral oil lubricant and for the remainder consisting of not exceeding 1 per cent of modifying agents to improve oiliness and coefficient of friction.

2. A non-spreading lubricant having a base consisting of 50 to 90 parts by weight of a non-spreading component and 50 to 10 parts of a spreading component, said components being compatible and intersoluble in one another; said non-spreading component consisting of a liquid homologous mixture of stable non-volatile polar aralkyl compounds each having an alkyl chain and a nuclear aromatic radical connected to said chain and including a strong non-anionic negative group, said non-spreading component demonstrating a positive contact angle with a steel surface in excess of 10 degrees and having a surface tension of at least 35 dynes per centimeter, the alkyl chain having from about 5 to 21 carbon atoms; said spreading component consisting of a liquid homologous mixture of stable non-volatile organic compounds each containing saturated aliphatic chains of 4 to 16 carbon atoms and at least two polar groups, of which one is the ester group and another is selected from the radicals consisting of the ester group and the aryl groups; said lubricant being further characterized in containing less than 5 per cent of mineral oil lubricant and for the remainder consisting of not exceeding 1 per cent of modifying agents to improve oiliness and coefficient of friction.

3. A non-spreading lubricant having a base consisting of 50 to 90 parts by weight of a non-spreading component and 50 to 10 parts of a

spreading component, said components being compatible and intersoluble in one another; said non-spreading component consisting of a liquid homologous mixture of stable non-volatile polar aralkyl compounds each being the ester of an aralkyl alcohol and an aralkyl acid and having an alkyl chain and a nuclear aromatic radical connected to said chain and including a strong non-anionic negative group, said non-spreading component demonstrating a positive contact angle with a steel surface in excess of 10 degrees and having a surface tension of at least 35 dynes per centimeter, the alkyl chain having from about 5 to 21 carbon atoms; said spreading component consisting of a liquid homologous mixture of stable non-volatile organic compounds each containing a saturated aliphatic chain of 4 to 16 carbon atoms and at least two polar groups of which two are ester groups; said lubricant being further characterized in containing less than 5 per cent of mineral oil lubricant and for the remainder consisting of not exceeding 1 per cent of modifying agents to improve oiliness and coefficient of friction.

4. A non-spreading lubricant having a base consisting of 50 to 90 parts by weight of a non-spreading component and 50 to 10 parts of a spreading component, said components being compatible and intersoluble in one another; said non-spreading component consisting of a liquid homologous mixture of stable non-volatile polar aralkyl compounds each being the ester of an aralkyl alcohol and an aralkyl acid having an alkyl chain and a nuclear aromatic radical connected to said chain, said non-spreading component demonstrating a positive contact angle with a steel surface in excess of 10 degrees and having a surface tension of at least 35 dynes per centimeter, the alkyl chain having from about 5 to 21 carbon atoms; said spreading component consisting of a liquid homologous mixture of stable non-volatile organic compounds each containing a saturated aliphatic chain of 4 to 16 carbon atoms and at least two polar groups of which two are ester groups; said lubricant being further characterized in containing less than 5 per cent of mineral oil lubricant and for the remainder consisting of not exceeding 1 per cent of modifying agents to improve oiliness and coefficient of friction.

5. A non-spreading lubricant as in claim 1, in which the non-spreading component mixture consists of aralkyl alcohol esters of aralkyl acids, said acids each having an alkyl chain of at least 3 carbon atoms; and in which the spreading component mixture consists of diesters of a glycol with monovalent saturated organic acid groups having said saturated aliphatic chain of 4 to 16 carbon atoms.

6. A non-spreading lubricant as in claim 1, having a pour point below minus 50 degrees F., in which the non-spreading component mixture consists of 50 to 70 parts by weight of benzyl phenylundecanoate; and the spreading component mixture consists of 30 to 50 parts of stable organic glycol diesters having the said saturated aliphatic carbon chain of 4 to 16 carbon atoms.

7. A non-spreading lubricant as in claim 1, in which the non-spreading component mixture consists of 50 to 70 parts by weight of benzyl phenylundecanoate; and the spreading component mixture consists of 30 to 50 parts by weight of diesters of a glycol with an aliphatic monovalent acid having the said saturated aliphatic chain of 4 to 16 carbon atoms.

8. A non-spreading lubricant as in claim 1, in which the non-spreading component mixture consists of benzyl phenylundecanoate; and the spreading component mixture consists of benzyl undecanoate.

9. A non-spreading lubricant as in claim 1, in which the non-spreading component mixture consists of aralkyl alcohol esters of aralkyl acids, said acids each having an alkyl chain of at least 3 carbon atoms; and said spreading component mixture consists of thioglycol diesters of saturated aliphatic acids each having at least 3 carbon atoms.

10. A non-spreading lubricant consisting essentially of 50 to 70 parts by weight of benzyl 15

phenylundecanoate and 30 to 50 parts of diethylene glycol dicaproate.

GEORGE E. BARKER.

#### REFERENCES CITED

The following references are of record in the file of this patent:

#### UNITED STATES PATENTS

| Number    | Name          | Date          |
|-----------|---------------|---------------|
| 2,179,067 | Smith         | Nov. 7, 1939  |
| 2,241,531 | Wiezevich     | May 13, 1941  |
| 2,355,616 | Barker        | Aug. 15, 1944 |
| 2,409,443 | Morgan et al. | Oct. 15, 1946 |